

Patented Jan. 9, 1940

2,186,719

# UNITED STATES PATENT OFFICE

2,186,719

## PHOTOGRAPHIC SILVER HALIDE EMULSIONS

Alfred Fröhlich and Wilhelm Schneider, Dessau, Germany, assignors, by mesne assignments, to Agfa Ansco Corporation, Binghamton, N. Y., a corporation of Delaware

No Drawing. Application November 18, 1937, Serial No. 175,285. In Germany December 18, 1936

11 Claims. (Cl. 95—6)

This invention relates to color photography and more particularly to a new and improved photographic material for color forming development.

In the manufacture of color transparencies and color picture by photography and cinematography it has been proposed to use silver halide emulsions containing dyestuff components. The mode of producing the color picture differs with the nature of the dyestuff components. In U. S. Patents Nos. 1,102,028 and 1,055,155 dyestuff components are used which yield dyestuff pictures with certain developers by color forming development. For producing multi-color pictures it has been proposed to cast several light-sensitive layers containing different coupling components one upon the other and in order to avoid diffusion of the coupling components the light-sensitive layers have been isolated from each other by intermediate layers. It has been shown, however, that this precaution does not prevent the diffusion to the extent required by practice. The problem has been solved by using dyestuff components which are fast to diffusion and for the first time a process has been attained by which a multi-layer film yields a color picture by a simple development process (see U. S. Patents 2,179,288, 2,178,612 and 2,179,244 and U. S. patent applications, Ser. No. 94,340 filed August 5, 1936, Ser. No. 159,518 filed August 17, 1937, Ser. No. 164,499 filed September 12, 1937). A further possibility of rendering dyestuff components fast to diffusion consists in introducing into their molecule a sterol radical or to link up the dyestuff component molecules in a chain like manner.

This invention has for an object to provide a new range of dyestuff components with improved properties.

A further object is the provision of silver halide emulsions having incorporated the new dyestuff components fast to diffusion.

A further object is the provision of silver halide emulsions having incorporated the new dyestuff components fast to diffusion in a dissolved form.

A further object is the provision of an improved film for color photography having superposed silver halide emulsion layers at least one of said layers containing a dyestuff component made fast to diffusion by the introduction into its molecule of a radical according to this invention.

Further objects will be seen from the detailed specification following hereafter.

The present invention is based on a process in which especially useful dyestuff formers fast to diffusion are obtained by introducing into the

molecule of a dyestuff intermediate product substituents which are radicals of hydro-aromatic or mixed aromatic-hydroaromatic or hydrogenated heterocyclic compounds. Such compounds are for example, 4-amino-4'-cyclohexyldiphenyl-ether, 2,4-diamino-4-cyclohexyl diphenyl-ether, 1-cyclohexyl-4-aminobenzene-5-sulfonic acid, para-amino-cyclohexylbenzene, aminotetraline, aminodecaline, amino-dicyclohexyl, 4-cyclohexyl benzoic acid, 4-cyclohexyl benzaldehyde, 6-amino-tetrahydroquinoline. The dyestuff component may be united to a body of this kind with the aid of a reactive atom or atom group which may be present in the hydrogenated ring, in the aromatic ring or in the hydrogenated heterocyclic ring. The several rings may also contain one or more of the substituents disclosed in the U. S. patents and U. S. patent applications referred to above. These substituents have already a tendency to make the molecule of the dyestuff component fast to diffusion. Dyestuff components into which the radical of the hydroaromatic or hydrogenated heterocyclic compound may be introduced are, for example,  $\alpha$ - and  $\beta$ -hydroxynaphthoic acids, 2,3-hydroxyanthracene carboxylic acid, salicylic acid, hydroxyfluorene carboxylic acid, 2,3-hydroxycarbazole carboxylic acid,  $\alpha$ -naphthol aldehyde, 1-amino-phenyl-3-methyl-5-pyrazolone, aromatic amines, aminonaphthols, aminonaphthol carboxylic acids, aminonaphthol sulfonic acids, aminophenols, aminobenzoyl acetic acid ester arylides, aminonaphthoyl acetic acid ester arylides, acyl acetic acid ester aminoarylides or the like. The components may also be built up from the said compounds which hinder diffusion, for example, the pyrazolone from 4-cyclohexyl phenyl hydrazine and ethyl acetacetate.

The dyestuff components used in the invention may be added to the emulsion at any point of its production. The silver halide emulsions thus obtained are especially suitable for the purpose of color photography and may be made into layers in known manner, being applied superimposed on each other on one or both sides of a support. They may be sensitized for various regions of the spectrum. Emulsions may be applied, however, in another manner, for example the several sensitized emulsions having the different dyestuff formers may be brought on to the support in the form of small particles. The emulsion layers used in the invention may be combined with other layers in which the color picture is produced by a different process, for example by mordant dyeing or by toning. Furthermore, the emulsion lay-

ers of the invention may be combined with other layers which contain other dyestuff formers fast to diffusion, as described in the U. S. patent applications cited hereunder.

5 The colored pictures may be produced in various manners, for example by the processes of U. S. Patents 2,179,228, 2,179,238, 2,178,612 and 2,179,244 and U. S. applications Serial No. 94,340 filed August 5, 1936, Ser. No. 141,093 filed May 6, 1937, Ser. No. 159,518 filed August 17, 1937 and 10 Ser. No. 164,499 filed September 18, 1937. Or the components located in multi-layer film may be converted into azo-dyes following development and fixing by treatment with a diazo compound such as a carbonic acid solution of tetrazotized 15 benzidine disulfonic acid. There is thus produced in each emulsion layer together with a silver picture a dyestuff in which no structure can be perceived by magnification. The film is then treated with a silver bleaching out bath, i. e. that 20 described in British Patent 401,340 to produce the dye image.

25 dye image.  
The exposed emulsion layers may be developed by a simple color forming development or by a reversal development as described in U. S. Patent  
2,179,234. The pictures may also be produced in  
30 multi-layer material, each layer containing one  
of said dyestuff components by exposing the ma-  
terial, developing to black and white in for in-  
stance Amidol, dissolving silver from the negative  
35 so produced by bleaching in for example a  
chromic acid bath, forming images in the re-  
maining silver halide, developing in a developer  
such as is used above, forming silver halide images  
by treatment in a bleaching bath 1. e. again of  
40 chromic acid, forming latent images, transform-  
ing the images into silver and color images in a  
developer capable of forming dyestuffs with said  
dyestuff component, removing the developed sil-  
ver and fixing in thiosulfate. In the production  
45 of color pictures the silver is generally completely  
removed. In the production of black-and-white  
pictures with the aid of the silver halide emulsion  
layers produced in accordance with this invention  
the silver may be removed or may remain in the  
layer.

The following examples illustrate the invention:

1. Ethylbenzoylacetate is condensed with 4-  
50 amino-phenyl-4'-cyclohexylbenzene:



When this body is added to a silver halide emulsion it remains fixed therein and when the emulsion has been exposed to light and developed by color forming development, a yellow picture is obtained. By operating with the known precautions by the anti-diazotate process there is also obtained a yellow dyestuff picture.

2. 1-aminophenyl - 3 - methyl-5-pyrazolone is condensed with 4-cyclohexyl benzoic acid chlo-

ride. A compound of the following formula results:



A silver halide emulsion which has received an addition of this body and has been worked up in manner similar to that described in Example 1 produces in the first case a red and in the second case a yellow dyestuff picture. 25

3. 2,3-hydroxynaphthoic acid chloride is condensed with 4,4'-dicyclohexylaniline:



A compound of the following formula results:



The silver halide emulsion to which this body has been added yields when exposed and developed by the anti-diazotate process a red dyestuff picture. 55

4. 2,3-hydroxycarbazole carboxylic acid chloride is condensed with 6-amino-N-ethyl-tetrahydroquinoline:



A compound of the following formula results:



5. 1-amino-5-naphthol is condensed with perhydrodiphenyl carboxylic acid:



10. A compound of the following formula results:



20. When this body is added to a photographic silver halide emulsion which is then exposed to light and developed by color forming development there is obtained a blue dyestuff picture. When the development is by the anti-diazotate process there is obtained according to the diazo-compound used a red to violet dyestuff picture.

25. 6.  $\alpha$ -hydroxynaphthoic acid chloride is condensed with perhydro-4-aminodiphenyl:



35. A compound of the following formula results:



50. When this body is added to a silver halide emulsion it is then exposed to light and after development treated with a solution of tetrazotized 3,3-dicarboxylic acid and then by the known silver bleaching out process there is obtained a blue-red azo-dyestuff picture.

What we claim is:

1. A silver halide emulsion for color photography containing a dyestuff component for color forming development having attached thereto by an acid amide linking a group having at least two organic rings, one of which at least is hydrogenated said group being capable of rendering said dyestuff component fast to diffusion in said silver halide emulsion.

2. A silver halide emulsion for color photography containing a dyestuff component for color forming development having attached thereto a

carboxylic acid radical the hydroxyl group of which is substituted by an amine radical having at least two organic rings, one of which at least is hydrogenated, said amine radical being capable of rendering said dyestuff component fast to diffusion in said silver halide emulsion.

3. A silver halide emulsion for color photography containing a dyestuff component for color forming development having attached thereto an amino group one hydrogen atom of which is substituted by the radical of an organic carboxylic acid having at least two organic rings one of which at least is hydrogenated said carboxylic acid radical being capable of rendering said dyestuff component fast to diffusion in said silver halide emulsion.

4. The silver halide emulsion defined in claim 1 wherein said two rings are selected from the class consisting of fused rings and rings linked together by a direct nuclear carbon to nuclear carbon linkage.

5. A silver halide gelatine emulsion for color photography containing a dyestuff component for color forming development having attached thereto by an acid amide linkage a group having at least 2,6-membered isocyclic rings linked together by a direct nuclear carbon to nuclear carbon linkage, at least one of said rings being hydrogenated, said group being capable of rendering said dyestuff component fast to diffusion in said silver halide emulsion.

6. The silver halide emulsion defined in claim 5, wherein said hydrogenated ring is cyclohexyl.

7. A silver halide gelatine emulsion for color photography containing a dyestuff component for color forming development having attached thereto by an acid amide linkage a group having 2 fused rings, one of which is heterocyclic and one of which is hydrogenated, said group being capable of rendering said dyestuff component fast to diffusion in said silver halide emulsion.

8. The silver halide emulsion defined in claim 7, wherein said group having 2 fused rings is a hydrogenated quinoline.

9. A silver halide gelatine emulsion for color photography containing a dyestuff component for color forming development fast to diffusion in said silver halide emulsion, said dyestuff component being the condensation product of ethylbenzoyl acetate with 4-amino-phenyl-4'-cyclohexylbenzene.

10. A silver halide gelatine emulsion for color photography containing a dyestuff component for color forming development which is fast to diffusion in said silver halide emulsion, said dyestuff component being a condensation product of 1-amino-phenyl-3-methyl-5-pyrazolone with 4-cyclohexyl-benzoic acid chloride.

11. A silver halide gelatine emulsion for color photography containing a dyestuff component for color forming development which is fast to diffusion in said silver halide emulsion, said dyestuff component being the condensation product of 2,3-hydroxy carbazole carboxylic acid chloride with 6-N-ethyl-aminotetrahydroquinoline.

ALFRED FRÖHLICH.  
WILHELM SCHNEIDER.